

Feb. 23, 1965

B. TARMANN

3,170,204

MOLD FOR THE CONTINUOUS CASTING OF HIGH-MELTING METALS

Filed Feb. 20, 1961



3,170,204  
MOLD FOR THE CONTINUOUS CASTING OF  
HIGH-MELTING METALS

Bruno Tarmann, Styria, Austria, assignor to Gebr. Böhler & Co. Aktiengesellschaft, Vienna, Austria  
Filed Feb. 20, 1961, Ser. No. 90,561  
Claims priority, application Austria, Feb. 25, 1960,  
1,448/60  
4 Claims. (Cl. 22—136)

It is known that molds for the continuous casting of high-melting metals such as iron and steel must consist of a material of high thermal conductivity and that the wall thickness of the molds must be sufficient to withstand the mechanical stresses to be expected.

If silver is left out of consideration among the materials of adequate thermal conductivity, copper is a material suitable in the first place for making the mold, and other materials will only be used when required for special reasons, e.g., when the material cast in the mold is to be subjected to electric induction. In such cases, a lower thermal conductivity of the mold material must be accepted.

Regarding structure, there are integral and composite molds. The composite molds are composed of plates whereas the integral molds consist of a prismatic or cylindrical tube. With respect to the cooling arrangement there are molds formed with cooling bores, and others surrounded by a water jacket. Regarding the wall thickness, there are thin-walled molds, the wall thickness of which is only sufficient for the mechanical stresses to be expected—the upper limit lies at about 20 millimeters—and thick-walled molds having wall thicknesses which exceed this value. In the case of cross-sections which are so large that a self-supporting wall thickness larger than 20 mm. would be required for mechanical reasons, supports and holders are required if the advantages of a thin-walled mold are to be retained.

Each type of mold has its advantages and disadvantages, which differ with the shape and size of the cross-section, the pouring rate and the kind of steel to be poured. For this reason, the molds employed in existing continuous casting plants vary within a wide range.

The durability of a mold for continuous casting is essential for its usefulness. The durability may be expressed by the number of casting cycles which can be performed without need for straightening or repairing the mold.

The high thermal loading of the mold for continuous casting results in high stresses being set up in the mold wall as a result of thermal expansion. In continuous operation, these stresses result in deformation, which adversely affects the contact between the skin of the billet and the mold wall and consequently reduce the dissipation of heat. When the deformation has reached such a degree that the formation of the skin is disturbed owing to an unsufficient dissipation of heat, the billet will show surface cracks and the durability of the mold is exhausted.

It has now been observed that these undesired deformations occur mainly in the neighborhood of the level of the molten material. This level varies in the mold within a range which can amount to  $\pm 30$  mm. even in a carefully controlled casting operation. It has also been observed that the molds are more liable to be subjected to deformation adjacent to the surface of the cast material as the heat transfer rate of the mold increases; this rate is known to depend to a high degree on the thermal conductivity of the material of the mold.

To eliminate these undesired phenomena, it would be desirable to provide a mold material having a thermal conductivity which is higher than that of copper, if possible.

Surprisingly, however, it has been found that the undesired deformation in the neighborhood of the level of the surface of the cast material can be avoided to a high degree if precipitation-hardened copper alloys are used which consist of more than 85% copper and at least one alloying element which enables precipitation hardening.

It was not foreseeable that success could be obtained in the present case by a measure which will necessarily reduce the thermal conductivity of copper.

10 Suitable alloying additions to the copper include mainly chromium, silicon, silver and beryllium. The amount of each of these materials should suitably not exceed 3%.

Such alloys known per se consist preferably of 1-2% Cr, with or without 0.1-1% Si, balance copper and impurities which are inevitable in the manufacturing process.

15 It is essential for the invention that the alloys which are recommended and known per se are used in a precipitation-hardened condition because only in this condition is the thermal conductivity not substantially less than that of pure copper whereas the yields point at elevated temperature and the creep stress are much higher than the corresponding values for pure copper.

20 The precipitation-hardening treatment of these known alloys with, e.g., 1.5% Cr is effected by a solution annealing at about 1000° C. followed by quenching in water and reheating for one to four hours at temperatures between 350° and 600° C., preferably by reheating for two hours at 400° C.

25 When welding operations are required during the manufacture of the mold, the precipitation-hardening treatment is suitably effected after the welding operation.

30 Molds according to the invention may consist partly or entirely of precipitation-hardened copper alloys.

35 Integral molds, which are in most cases subject to very high stresses, consist in condition ready for installation preferably entirely of a precipitation-hardened copper alloy owing to the simpler manufacture.

40 On the other hand, it may be suitable in the case of composite molds composed of plates to use the precipitation-hardenable copper alloys only in the region where high stresses occur, mainly adjacent to the surface of the molten material. In that case the other parts of the mold consist of pure copper, as before.

45 The durability of molds for continuous casting according to the invention is under comparable conditions in all previously observed cases a multiple of that of usual copper molds.

50 The subject matter of the invention will be described more in detail with reference to an illustrative embodiment. The drawing shows a mold for continuous casting. The mold 1 consisting of the alloy according to the invention is provided at both ends with flanges 2 or 3, the material of which need not consist of the alloy according to the invention but must be capable of being joined to the body of the mold without a gap. Besides, the mold 55 is surrounded by a jacket 4, which serves to receive the cooling water for cooling the wall of the mold and causing the solidification of the melt poured into the mold to the level L indicated by a broken line.

55 60 What is claimed is:

65 1. A mold for the continuous casting of metals, said mold consisting of a precipitation hardened copper alloy at the level of molten material, said alloy consisting essentially of about 1% to 2% chromium, incidental impurities and the balance being copper; and copper metal in the other level.

70 2. A mold for the continuous casting of metals, said mold consisting of a precipitation hardened copper alloy at the level of molten material, said alloy consisting essentially of about 1% to 2% chromium, 0.1% to 1% silicon, incidental impurities and the balance being copper; and copper metal in the other level.

3. A mold for the continuous casting of metals, said mold consisting of a precipitation hardened copper alloy at least at the level of molten material, said alloy consisting essentially of about 1% to 2% chromium, incidental impurities and the balance being copper.

4. A mold for the continuous casting of metals, said mold consisting of a precipitation hardened copper alloy at least at the level of molten material, said alloy consisting essentially of about 1% to 2% chromium, 0.1% to 1% silicon, incidental impurities and the balance being copper.

10

#### References Cited by the Examiner

##### UNITED STATES PATENTS

|           |      |             |       |           |
|-----------|------|-------------|-------|-----------|
| 2,192,497 | 3/40 | Hessenbruch | ----- | 75—160    |
| 2,547,129 | 4/51 | Klement     | ----- | 75—153 XR |
| 2,944,309 | 7/60 | Schaaber    | ----- | 22—136 XR |

MICHAEL V. BRINDISI, *Primary Examiner.*

MARCUS U. LYONS, RAY K. WINDHAM, NEDWIN BERGER, *Examiners.*